

## UNITED STATES PATENT OFFICE

2,334,076

## LUBRICANT FOR SPLIT DIES

Samuel Epstein, Bethlehem, and John R. Kreiser, Lebanon, Pa., assignors to Bethlehem Steel Company, a corporation of Pennsylvania

No Drawing. Application September 16, 1941,  
Serial No. 411,016

6 Claims. (Cl. 252—22)

This invention relates generally to the manufacture of wire, rod, nails, carriage bolts, screws and the like, and more particularly to lubricants especially adapted for forming such articles in split or open dies.

Standard carriage bolts have round unslotted heads and square necks, although special types are also made with bevel, countersunk or askew heads or ribbed necks. The enlarged necks are characteristic of these bolts, yet with ordinary die lubricants it is difficult to fill them out properly to obtain sharp, unrounded edges.

The split or open die used in cold-heading carriage bolts and the like is made in two pieces, so that the die opening may "breathe" or give slightly to prevent sticking of the work-piece. Before entering the die the wire is cleaned, coated with lime, and covered with a suitable lubricant to protect the wire and die surfaces.

For a long time it has been known that dropping a bit of oil on the wire as it went into the heading die would cause rounded instead of sharply filled out edges on the necks of carriage bolts. That is why oil cannot be used as an additional lubricant on such work. The rounding of the edges is generally attributed to oil being trapped and forming pockets in the die crevices. However, even very minute amounts of oil produce the effect. From this and other evidence, it has been concluded that another phenomenon also plays an important part. It is that the oil causes the work to slip too easily so that it is not gripped positively by the die surfaces, and hence cannot fill out the die properly. The effect is similar with a dry lubricating coating too high in lubricating value. The wire is too slippery and the necks are not filled out well. A better filled out neck is obtained with a less slippery coating on the wire.

A less slippery coating not only gives better filled out necks, but also better filled out and rounded heads. This is especially important for wood screws. It also gives a wire which is held more positively in nail making machines, so that a more evenly pointed nail is cut by the dies with less "whiskering." Such wire also works better in cut-off machines for spring wire, due to less slippage in the guide rolls, so that more even lengths are obtained and more uniform springs.

Various recourse have hitherto been tried to get a well-filled out neck. Thus "bright" drawn wire, with no coating at all has been used. This gives a well-filled out neck but leaves the heading operation without lubrication and does not protect the wire from rusting. A heavier sul

coating is generally used for this type of work, particularly for nail wire, the sul or rust coating being applied by holding the rod in a fine water spray after washing and before liming the rod. The heavier sul decreases the slipping but it also increases the die wear. Furthermore, it is difficult to obtain a uniform coating of sul as this may vary considerably from coil to coil and within the same coil. Thinner lime may avoid undue clogging in the dies and give a better filled out neck; also because less lubricant is taken up by thinly limed rod the coating may be less slippery. An additional pass through the drawing die also makes for a thinner and less slippery coating. 15 This is, of course, expensive.

One object of our invention, therefore, is to provide an improved lubricant for split die work.

Another object is to give better filled out necks to carriage bolts and the like.

A further object is to produce more fully rounded heads on wood-screws and the like.

Still a further object is a lubricant which results in better and more uniformly pointed nails, and in less slippage in the guide rolls of spring wire cut-off machines.

Other objects, purposes and advantages of this invention will more clearly appear in the following pages of the specification and in the appended claims, and we now set forth in detail the particulars of our invention.

We have found by experiment that adding an ingredient to the die lubricant which makes for less slipperiness, calcium resinate for instance, definitely gives the most uniform and dependable results with split dies.

The addition of about 8 per cent of calcium resinate by weight will improve any lubricant ordinarily used with split dies, but we have found the following mixture, in approximate parts by weight, to be quite the best for the purpose:

|                  |          |
|------------------|----------|
| Calcium resinate | 2 to 3   |
| "Acrawax C"      | 2 to 4   |
| Hexachlorbenzene | 10 to 12 |
| Graphite         | 5 to 6   |

All the components in this lubricant are dry and water repellent, with sufficiently high melting points not to cause smearing or caking in the dies, and all except calcium resinate have high lubricating values. Even calcium resinate, although not a particularly good lubricant, is a soft material, and has no abrasive effect such as lime, for example, sometimes has. The calcium resinate makes for a drier and less slippery wire which aids materially in filling out the neck.

The substance of lowest melting point herein, the synthetic wax "Acrawax C" (cetyl acetamide, melting point, 275° F.), helps to spread the lubricant over the limed wire. Natural waxes or wax-like substances of approaching melting points, such as ozokerite or montan or carnauba wax, or blends thereof, may be substituted in equal proportions for this ingredient. Hexachlorbenzene, melting point, 440° F., has good lubricating properties and is water repellent. The graphite also lubricates, gives a distinctive pleasing sheen, and aids in maintaining a stable lustrious coating in shipment and storage.

If the darker color due to the graphite is not desired, the finished bolts may be tumbled and blued or otherwise conventionally processed to remove or change the color, or the following white lubricating mixture may be used, in parts by weight

|                          |    |
|--------------------------|----|
| Hydrated lime            | 18 |
| "#1 Penola V. D." grease | 5  |
| Calcium resinate         | 2  |

The above-mentioned "#1 Penola V. D." grease is an ordinary lime-base grease such as is used in drawing wire, and other greases of this type may be substituted as desired.

The thinner coating produced by these lubricants is a factor which aids in giving a well-filled-out neck, and also provides a significant saving in the quantity and cost of lubricant used for a given amount of work.

Although we have shown and described our invention in considerable detail, we do not wish to be limited to the exact and specific materials and details shown and described, but may use such substitutions, modifications or equivalents

thereof as are within the scope of the invention and claims.

Having thus described our invention, what we claim as new and useful and desire to secure by Letters Patent is:

1. A lubricant for use in the manufacture of wire springs, nails, bolts, screws and the like comprising, in approximate parts by weight, 2 to 3 calcium resinate, 2 to 4 wax of melting point approximately 275° F., 10 to 12 hexachlorbenzene, and 5 to 6 graphite.

10 2. A lubricant for use in the manufacture of wire springs, bolts, screws and the like comprising, in approximate parts by weight, 2 to 3 calcium resinate, 2 to 4 montan wax, 10 to 12 hexachlorbenzene, and 5 to 6 graphite.

15 3. A lubricant for use in the manufacture of wire springs, bolts, screws and the like comprising, in approximate parts by weight, 2 to 3 calcium resinate, 2 to 4 carnauba wax, 10 to 12 hexachlorbenzene, and 5 to 6 graphite.

20 4. A lubricant for use in the manufacture of wire springs, bolts, screws and the like comprising, in approximate parts by weight, 2 to 3 calcium resinate, 2 to 4 cetyl acetamide, 10 to 12 hexachlorbenzene, and 5 to 6 graphite.

25 5. A lubricant for split dies comprising, by weight, approximately 2 parts calcium resinate, 4 parts cetyl acetamide, 10 parts hexachlorbenzene, and 5 parts graphite.

30 6. A lubricant for use in the manufacture of wire springs, nails, bolts, screws and the like comprising a mixture of calcium resinate, hexachlorbenzene, wax having a melting point approaching 275° F. and graphite.

SAMUEL EPSTEIN.  
JOHN R. KREISER.